

May 17, 1932.

J. J. DUNN

1,858,920

METHOD OF MAKING SEAMLESS TUBES

Filed March 23, 1928



*Fig. 1.*



*Fig. 2.*



*Fig. 3.*

*Inventor:*  
J. JAY DUNN,

*by:*  
D. Anthony Usina  
*his Attorney.*

## UNITED STATES PATENT OFFICE

JERRY JAY DUNN, OF ELLWOOD CITY, PENNSYLVANIA, ASSIGNOR TO NATIONAL TUBE COMPANY, OF PITTSBURGH, PENNSYLVANIA, A CORPORATION OF NEW JERSEY

## METHOD OF MAKING SEAMLESS TUBES

Application filed March 23, 1928. Serial No. 264,063.

This invention relates to a method of making seamless tubes of relatively large diameters, and has for its object the provision of a novel method by which seamless tubes of 5 over five and one-half inches finished diameter and less than one-half inch wall thickness may be commercially produced with a minimum amount of scrap.

With the methods heretofore generally 10 employed, the making of tubes of over five and one-half inches finished diameter and less than one-half inch wall thickness was commercially wasteful, due to the stresses which were set up in the metal. These 15 stresses caused the metal to tear and open up and the tubes, thus damaged, formed scrap which was useless.

The method for making seamless tubes in 20 general use in the United States, is to pierce a solid blank in a cross-roll machine, producing a tube somewhat less than one-fourth inch heavier than that of the finished wall desired; then rolling this heavy walled tube in a groove and over a mandrel in a two-high 25 rolling mill to reduce the wall thickness to the finished dimension; then passing the tube through a cross-roll machine for the purpose of removing the scratches left on the surfaces of the tube by the preceding operation, 30 rounding the tube and smoothing the surface generally; then sizing the tube.

An attempt has been made to modify this 35 method so as to produce large diameter tubes as disclosed in the patent to Ralph C. Stiefel, No. 1,474,800, dated November 20, 1923. In this Stiefel patent the usual steps are carried out except that a portion of the work 40 heretofore done in the piercing and rolling steps has been transferred to the cross-rolling step, where usually relatively little work is done.

The method of this Stiefel patent is objectionable due to the fact that too great an 45 amount of work must be done in the piercing operation and, due to the fact that the diameter of the pierced blank is reduced in the plug-mill operation, thereby increasing the amount of expansion that must be made in the 50 cross-rolling operation and, since there is a limit to the amount of expansion that can be

made in the cross-rolling operation, the size or diameter of the tubes is limited.

The present method consists in piercing a solid heated blank by cross-rolling over a 55 piercing plug so as to form a tubular blank materially longer and having a diameter slightly greater than that of the solid blank and a wall thickness of more than three times the thickness of the finished tube. During 60 this piercing operation, the work is limited so that a line on the blank, or an element 65 of its surface, will not be twisted or displaced a total, arithmetically added, an angle of twenty-five degrees; or, if the displacement is in one direction continuously, the total 70 should not exceed eighteen degrees. This is an important limitation since, if the twisting of the metal is held approximately within these limits, the metal will not tear and the 75 seams will not be opened.

After being pierced, the tubular blank is then immediately passed, without reheating, to a second piercing or cross-rolling, expanding operation. The once pierced tube is sufficiently hot to be easily worked and is subjected to a second piercing or cross-rolling, 80 expanding operation by again cross-rolling it over a conical piercing plug of materially greater size than the plug used in the first 85 piercing operation. This second piercing or cross-rolling, expanding operation is controlled so as to very materially increase the diameter and length of the blank while reducing the wall thickness to approximately twice the thickness of the wall of the finished 90 tube. The work in this second operation is also limited so as to prevent a line on the blank or an element of its surface being twisted or displaced an angle of more than fifteen degrees, thereby preventing the tearing of the 95 metal.

The blank, after the second piercing or cross-rolling operation, is then passed immediately and without reheating to an expanding, cross-rolling operation where it is 95 cross-rolled over an expanding plug to reduce the wall thickness from forty to sixty percent and to increase the diameter of the blank not less than thirty percent in reaching 100 the diameter of the finished tube, or, if the

- tube is to be sized, to a slightly greater diameter than the diameter of the finished tube. The length of the tube is also slightly increased in this cross-roll, expanding operation. The tube blank has sufficient ductility when entering this last operation that it will withstand more twist without tearing than it will in the piercing operations. Therefore, the work in the cross-roll, expanding operation is controlled so as to prevent the twisting or displacement of a line on the blank or an element of its surface more than thirty-five degrees.
- The tube, as produced by this last cross-rolling and expanding step, is suitable for use as a hot finished seamless tube. However, if desired, it may be passed through the well known reeling and sizing rolls to smooth and reduce it to exactly the desired diameter.
- Where superior finish is desired, the hot finished tube produced by the above described operations may be cold drawn in the usual way.

It will also be understood that I do not wish to be limited to the single expanding, cross-rolling operation since, when it is desired to produce some sizes of tubes, it may be necessary or desirable to use two or more expanding, cross-rolling operations, in which case the tube will preferably be reheated after the first expanding, cross-rolling operation. It may also be desirable, when producing extremely thin-walled tubes, to reheat the blanks after the second piercing or cross-rolling operation and, therefore, I do not wish to be limited to expanding without reheating.

A particular advantage is gained by the method of this application in that the diameter of the blank is increased at each operation, and also by the fact that only three passes are generally necessary to produce a hot finished tube while, in the methods of the prior art in which plug-mills are used to reduce the wall thickness, the diameter of the blank is reduced and several passes are required in the plug-mill which cools the tube to such a degree that the work of the expanding cross-rolls is limited.

In the drawings:

Figure 1 is a diagrammatic view showing the first piercing operation.

Figure 2 is a similar view showing the second piercing or cross-rolling operation.

Figure 3 is a similar view showing the expanding operation.

Referring more particularly to the drawings in which the apparatus is diagrammatically shown performing the steps of this invention, the letter A designates the solid heated blank which is being pierced in a standard piercing mill composed of cross-rolls 2 and a piercing plug 3. The rolls 2 are provided with the usual pass and serve to force the blank over the piercing point 3 so

as to pierce and somewhat expand the blank forming a relatively thick-walled tubular blank.

The relatively thick-walled tubular blank designated by the letter B is next passed to a second standard piercing mill, shown in Figure 2, composed of cross-rolls 5 and a tapered piercing plug 6 of materially greater diameter than the inner diameter of the blank. The rolls 5 are provided with the usual pass and serve to force the tubular blank over the piercing point 6 so as to again pierce or expand the blank and reduce its wall thickness materially, thus forming a tubular blank having a materially greater diameter and thinner wall than the blank produced in the first piercing operation.

The work in each of the above piercing operations is limited so as not to twist the metal blank a sufficient amount to tear or rupture the metal and yet is sufficiently heavy so as to produce a blank, after the second piercing operation, having a wall of approximately twice the thickness of the wall of the finished tube.

Experience has shown that the work in the first piercing operation should be limited so as not to twist a line on the blank or an element of its surface in one direction continuously more than 18 degrees, while the work in the second piercing operation should be limited so as not to twist a line on the blank or an element of its surface in one direction more than 15 degrees, so as to prevent tearing or rupturing of the metal.

The blank C produced by the second piercing operation is passed immediately, without reheating, from the second piercing operation to a cross-rolling and expanding mill, shown in Figure 3, and composed of cross-rolls 8 and an expanding plug 9 of standard design. The rolls 8 are provided with the usual pass and serve to force the blank C over the expanding plug 9 so as to expand the blank more than thirty percent and, at the same time, reduce the wall thickness from 40 to 60 percent, thus forming a relatively thin-walled large diameter tube in three cross-roll passes.

The work of the cross-rolling and expanding mill is limited or controlled so as not to twist a line on the blank or an element of its surface in one direction more than 35 degrees so as to prevent tearing or rupturing of the metal in this last pass.

By utilizing the three cross-rolling operations, as above described, by which a tube is formed in the first operation and the tube is expanded and its wall reduced in each of the other two operations, I am enabled to materially reduce the number of passes over the number of passes necessary when a plug-mill is used to reduce the wall thickness and, therefore, the tubular blank is delivered to the last expanding operation sufficiently hot

to permit the maximum expansion of diameter and reduction of wall thickness.

While I have described certain specific steps and limitations in the carrying out of such steps of my method, and also have illustrated certain apparatus suitable for performing the steps of my method, it will be understood that I do not wish to be limited thereto since various modifications may be carried out and details of the apparatus changed without departing from the scope of my invention as defined in the appended claims.

I claim--

1. The method of making large diameter seamless tubes which consists in piercing a solid heated blank by cross-rolling over a piercing plug to form a tubular blank having a diameter slightly greater than that of the solid blank and a wall thickness less than twenty percent of the outside diameter, then subjecting said tubular blank without reheating to a second piercing operation by cross-rolling over a piercing plug to very materially increase the diameter and length and decrease the wall thickness of the blank, and then subjecting the tubular blank resulting from said second piercing operation without reheating to a cross-rolling operation over an expanding plug so as to reduce the wall thickness not less than forty and not more than sixty percent of the wall thickness of the tubular blank resulting from the second piercing operation and also cause a relatively large increase in the diameter of the tube and a relatively slight increase in length. 80
2. The method of making large diameter seamless tubes which consists in piercing a solid heated blank by cross-rolling over a piercing plug to form a tubular blank having a diameter slightly greater than that of the solid blank and a wall thickness less than twenty percent of the outside diameter, then subjecting said tubular blank without reheating to a second piercing operation by cross-rolling over a piercing plug, controlling the work in said cross-rolling operation so as to prevent the twisting of a line on the blank in one direction continuously more than 18 degrees and to form a tubular blank having a diameter slightly greater than that of the solid blank and a wall thickness of more than three times the thickness of the wall of the finished tube, then subjecting said tubular blank without reheating to a second piercing operation by cross-rolling over a piercing plug, controlling the work in said cross-rolling operation so as to prevent the twisting of a line on the tubular blank in one direction continuously more than 15 degrees and to very materially increase the diameter and length of the tubular blank and to decrease the wall thickness of the blank to approximately twice the thickness of the wall of the finished tube, and then subjecting said tubular blank without reheating to a cross-rolling operation over an expanding plug, controlling the work in said cross-rolling operation so as to prevent the twisting of a line on the tubular blank in one direction more than 35 degrees, reduce the wall thickness not less than forty and not more than sixty percent of the wall thickness of the tubular blank, increase the diameter of the tubular blank not less than thirty percent, and also causing a change in the length of the blank inversely proportional to the change in its cross-sectional area. 100
3. The method of making large diameter seamless tubes which consists in piercing a solid heated blank by cross-rolling over a
4. The method of making large diameter seamless tubes which consists in piercing a solid heated blank by cross-rolling over a piercing plug, controlling the work in said cross-rolling operation so as to prevent the twisting of a line on the blank in one direction continuously more than 18 degrees and to form a tubular blank having a diameter slightly greater than that of the solid blank and a wall thickness of more than three times the thickness of the wall of the finished tube, then subjecting said tubular blank without reheating to a second piercing operation by cross-rolling over a piercing plug, controlling the work in said cross-rolling operation so as to prevent the twisting of a line on the tubular blank in one direction continuously more than 15 degrees and to very materially increase the diameter and length of the tubular blank and to decrease the wall thickness of the blank to approximately twice the thickness of the wall of the finished tube, and then subjecting said tubular blank without reheating to a cross-rolling operation over an expanding plug, controlling the work in said cross-rolling operation so as to prevent the twisting of a line on the tubular blank in one direction more than 35 degrees, reduce the wall thickness not less than forty and not more than sixty percent of the wall thickness of the tubular blank, increase the diameter of the tubular blank not less than thirty percent, and also causing a change in the length of the blank inversely proportional to the change in its cross-sectional area. 110
5. The method of making large diameter seamless tubes which consists in piercing a solid heated blank by cross-rolling over a piercing plug, controlling the work in said cross-rolling operation so as to prevent the twisting of a line on the blank in one direction continuously more than 18 degrees and to form a tubular blank having a diameter slightly greater than that of the solid blank and a wall thickness of more than three times the thickness of the wall of the finished tube, 120
6. The method of making large diameter seamless tubes which consists in piercing a solid heated blank by cross-rolling over a

then subjecting said tubular blank to a second piercing operation by cross-rolling over a piercing plug, controlling the work in said cross-rolling operation so as to prevent the twisting of a line on the tubular blank in one direction continuously more than 15 degrees and to very materially increase the diameter and length of the tubular blank and to decrease the wall thickness of the blank to approximately twice the thickness of the wall of the finished tube, and then subjecting said tubular blank to a cross-rolling operation over an expanding plug, controlling the work in said cross-rolling operation so as to prevent the twisting of a line on the tubular blank in one direction more than 35 degrees, reduce the wall thickness not less than forty and not more than sixty percent of the wall thickness of the tubular blank, increase the diameter of the tubular blank not less than thirty percent, and also causing a change in the length of the blank inversely proportional to the change in its cross-sectional area.

6. The method of making large diameter seamless tubes which consists in piercing a solid heated blank by cross-rolling over a piercing plug to form a tubular blank having a diameter slightly greater than that of the solid blank and a wall thickness less than twenty percent of the outside diameter, then subjecting said tubular blank to a second piercing operation by cross-rolling over a piercing plug to very materially increase the diameter and length and decrease the wall thickness of the blank, and then subjecting the tubular blank resulting from said second piercing operation to a cross-rolling operation over an expanding plug so as to reduce the wall thickness not less than forty and not more than sixty percent of the wall thickness of the tubular blank resulting from the second piercing operation and also cause a relatively large increase in the diameter of the tube and a relatively slight increase in length.

45 7. The method of making large diameter seamless tubes which consists in piercing a solid heated blank by cross-rolling over a piercing plug to form a tubular blank having a diameter slightly greater than that of the solid blank and a wall thickness less than twenty percent of the outside diameter, then subjecting said tubular blank to a second piercing operation by cross-rolling over a piercing plug to very materially increase the diameter and length and decrease the wall thickness of the blank, and then subjecting the tubular blank resulting from said second piercing operation to a cross-rolling operation over an expanding plug so as to reduce the wall thickness not less than forty and not more than sixty percent of the wall thickness of the tubular blank resulting from the second piercing operation, increase the diameter of the tube not less than thirty percent of the diameter of the tubular blank resulting from

the second piercing operation, and also causing a change in the length of the tube inversely proportional to the change in its cross-sectional area.

8. The method of making large diameter 70 seamless tubes which consists in piercing a solid heated blank by cross-rolling over a piercing plug, controlling the work in said cross-rolling operation so as to prevent the twisting of a line on the blank in one direction continuously more than 18 degrees and to form a tubular blank having a diameter slightly greater than that of the solid blank and a wall thickness of more than three times the thickness of the wall of the finished tube, then subjecting said tubular blank to a second piercing operation by cross-rolling over a piercing plug, controlling the work in said cross-rolling operation so as to prevent the twisting of a line on the tubular blank in one direction continuously more than 15 degrees and to very materially increase the diameter and length of the tubular blank and to decrease the wall thickness of the blank to approximately twice the thickness of the wall of the finished tube, and then subjecting said tubular blank to a cross-rolling operation over an expanding plug, controlling the work in said cross-rolling operation so as to prevent the twisting of a line on the tubular blank in one direction more than 35 degrees, reduce the wall thickness not less than forty and not more than sixty percent of the wall thickness of the tubular blank, increase the diameter of the tubular blank not less than thirty percent, and also causing a change in the length of the blank inversely proportional to the change in its cross-sectional area.

In testimony whereof, I have hereunto set my hand.

J. JAY DUNN.

105

110

115

120

125

130